# EUROPEAN PATENT SPECIFICATION

(11) **EP 2 986 749 B1**
(45) Date of publication and mention of the grant of the patent: **21.03.2018**
(21) Application number: 14717774.5
(22) Date of filing: 15.04.2014
(51) Int. Cl.: C21D 8/02, C22C 38/02, C22C 38/06, C21D 9/46, C22C 38/00, C22C 38/04, C22C 38/16

(54) **COLD REDUCED ENAMELLING STEEL SHEET, METHOD FOR ITS PRODUCTION, AND USE OF SUCH STEEL**
KALTGEWALZTES EMAILLIERTES STAHLBLECH, VERFAHREN ZU SEINER HERSTELLUNG, UND VERWENDUNG EINES SOLCHEN STAHLS
FEUILLE D'ACIER À ÉMAILLAGE RÉDUIT À FROID, SON PROCÉDÉ DE PRODUCTION ET UTILISATION D'UN TEL ACIER

(30) Priority: 15.04.2013 EP 13001949
(43) Date of publication of application: 24.02.2016
(73) Proprietor: Tata Steel IJmuiden BV, 1951 JZ Velsen-Noord (NL)
(72) Inventor: VAN KREVEL, Joost Willem Hendrik, NL-1970 CA IJmuiden (NL); VAN DUIJN, Ronald, NL-1970 CA IJmuiden (NL)
(74) Representative: Kruit, Jan
(86) International application number: PCT/EP2014/057601
(87) International publication number: WO 2014/170315

(56) References cited:
- EP-A1- 1 233 079
- US-A- 5 855 696
- Wikipedia: "Whiteboard - History", , 26 August 2013 (2013-08-26), XP002711937, Retrieved from the Internet: URL:http://en.wikipedia.org/wiki/Whiteboar d [retrieved on 2013-08-29]
- Jared L. Sommer: "Low-Cost Enamel Coatings on Stainless Steel Foil for Thin Film Photovoltaics", , 31 December 2002 (2002-12-31), XP002711938, Retrieved from the Internet: URL:http://www.sbir.gov/sbirsearch/detail/ 311030 [retrieved on 2013-08-29]

## Description

The invention relates to cold reduced vitreous enamelling steel sheet. The invention also relates to a method for producing an enamelled steel sheet and the use of such a steel sheet.

Cold reduced enamelling steel sheet is frequently used to fabricate products such as domestic appliances. During fabrication of such products, the steel sheet material is usually coated with an enamel layer. It is then desirable to obtain an enamel layer with good adhesion to the steel sheet, and with at most only a few visible defects such as fish scaling patterns. It is known that the resistance to fish scaling formation can be improved by a synergistic effect of boron and nitrogen content in cold reduced steel sheet.

Such an enamelling steel sheet is for instance known from EP1233079 and EP 1336665. The cold reduced enamelling steel sheet according to EP1336665 comprises (in weight ppm unless otherwise indicated) $5 \leq C \leq 90 ;$ $0.10 \leq Mn \leq 0.50 \left(wt . %\right) ;$ ${Al}_{as} \leq 300 \left(acid soluble Al\right) ;$ $O \leq 35 ;$ $S \leq 350$ $30 \leq N \leq 110 ;$ ${B}_{min} \leq B \leq {B}_{max} ;$ wherein ${B}_{min} = N \times 0.80 \times 10.8 / 14 {and B}_{max} = N \times 10.8 / 14 + 83 / 6 ;$ $50 \leq P \leq 160 ;$ in combination with ${Cu}_{min} \leq Cu \leq {Cu}_{max} ;$ wherein ${Cu}_{min} = P \times 1.00 \times 63.6 / 31 {and Cu}_{max} = P \times 2.00 \times 63.6 / 31 ;$ optionally $Si \leq 190 ;$ in each case the balance being Fe and unintentional and/or inevitable impurities.

Herewith is provided an enamelling steel sheet with a minimum of alloying elements that has deep drawing and/or bending properties which are sufficiently good, that is not too hard and can be handled in coil to coil enamel processing, while fish scale free. After applying and firing (white) enamel, the sheet is essentially free from fish scaling defects, and the enamel adhesion is satisfactory, if necessary by applying proper surface pretreatment and/or pretreatment layers. The reasons for the use of these elements in the quantities as specified is given in the above mentioned document.

However, it has been found that fish scaling defects free enamelled steel sheet can not be produced for all gauges.

It is therefore an object of the invention to provide enamelling steel in gauges that so far are not available.

It is also an object of the invention to provide a method for producing an enamelling steel sheet with the required gauges.

Moreover, it is an object of the invention to use such enamelling steel for specific purposes.

According to a first aspect of the invention a cold reduced enamelling steel sheet is provided, comprising (in weight ppm unless otherwise indicated) $5 \leq C \leq 90 ;$ $0.10 \leq Mn \leq 0.50 \left(wt . %\right) ;$ ${Al}_{as} \leq 300 \left(acid soluble Al\right) ;$ $O \leq 35 ;$ $S \leq 350 ;$ $30 \leq N \leq 110 ;$ ${B}_{min} < B \leq {B}_{max} ;$ wherein ${B}_{min} = N \times 0.80 \times 10.8 / 14 {and B}_{max} = N \times 10.8 / 14 + 144 / 6 ;$ $50 \leq P \leq 160 ;$ in combination with ${Cu}_{min} \leq Cu \leq {Cu}_{max} ;$ wherein ${Cu}_{min} = P \times 1.00 \times 63.6 / 31 {and Cu}_{max} = P \times 2.00 \times 63.6 / 31$ and optionally $Si \leq 190 ;$ the balance being Fe and unintentional and/or inevitable impurities,
wherein the steel sheet has been continuous annealed, and
wherein the steel sheet has a thickness between 0.10 mm and 0.34 mm.

The inventors have found that thinner gauges than the gauges possible so far can be used by using a continuous annealing process instead of the batch annealing process used so far. It has been common practice to batch anneal full hard enamelling steel for several days at a temperature between 620 and 680 °C. However, gauges thinner than 0.4 mm could not be used due to the appearance of fish scaling defects due to insufficient hydrogen retention. The inventors have found that continuous annealing improves the hydrogen retention of the steel. Using continuous annealing thus makes it possible to produce cold reduced enamelling steel sheet having gauges between 0.10 and 0.34 mm.

It is possible to produce the steel sheet such that it has a thickness between 0.12 and 0.34 mm, preferably between 0.15 mm and 0.32 mm, more preferably between 0.20 mm and 0.30 mm.

According to a preferred embodiment the steel has a maximal hardness of 85 - 130 micro Vickers with a load of 500 gram. The micro Vickers hardness is measured using a diamond tip which is pressed into the steel with a load of 500 gram. The hardness of the steel is thus such that that the steel has a good resistance against indentation, while the formability is satisfactory and strain build up during coil to coil enamelling is minimal.

Preferably the value for Bₘₐₓ = N×10.8/14 + 83/6. Herewith the mechanical properties are particularly optimised for relatively high Si content, i.e. in the range of 40 weight-ppm to 190 weight-ppm.

It is preferred that Bₘᵢₙ = Nx0.90x 10.8/14. Herewith the atomic ratio B/N is higher than 0.90. Herewith it is better assured that all nitrogen is indeed precipitated with B.

It is more preferred that Bₘᵢₙ = N×1.00×10.8/14. Herewith the atomic ratio B/N is higher than 1.00. It has been found that a small excess of B can be tolerated regarding the mechanical properties, with the advantage that it ensures that all N is indeed precipitated. Herewith the formation of fish scales is essentially fully suppressed.

In an embodiment, the steel sheet comprises: 45 ≤ N ≤ 110. The formation of fish scale defects has been found to be suppressed better if the amount of N present in the steel sheet is at least 45 ppm.

In an embodiment, the steel sheet comprises less than 89 ppm N. It has been found that the amount of added B can then be reduced while the formation of fish scale defects is nevertheless sufficiently reduced.

In an embodiment wherein the steel sheet comprises less than 89 ppm N, it is preferred that Bₘₐₓ = N×1.20×10.8/14. By keeping the atomic ratio B/N smaller than or equal to 1.20, the mechanical properties are kept close to their optimum. It is more preferred to keep the atomic ratio B/N smaller than or equal to 1.10. Herewith it is even better assured that no deteriorating effect on the mechanical properties results from the B addition. In addition, the steel remains free of defects that may affect the surface appearance of the surface finish as specified in norm EN 14864.

In a preferred embodiment, the maximum amount of C in the steel sheet is 50 ppm by weight. Herewith the ageing properties are better suited. In a more preferred embodiment, the maximum amount of C is 40 ppm. In a yet more preferred embodiment, the amount of C in the steel sheet is lower than 30 ppm by weight. Herewith, the strengthening of the steel sheet by ageing is maximised while no carbon boiling occurs during enamelling at 800 - 830° C.

In an embodiment of the invention, the steel sheet as described above has a grain size according to ASTM of 11 units or less. Herewith the desired mechanical properties and the pickling properties are achieved.

In an embodiment, the yield strength is between 140 MPa and 300 MPa, the tensile strength is between 270 MPa and 450 MPa, and the elongation to fracture is at least 30 %, all numbers measured in cross sectional direction to rolling in annealed, unaged and 1 % temper rolled condition. With these mechanical properties, the thin gauge enamelling steel is sufficiently suited for coil to coil enamelling without building up too much strain, and the thin gauge enamelling steel is also potentially well suited for light deep drawing applications. The steel sheet can have an *r*-value (at 90° to rolling direction) of higher than 1.0, and/or an *n*-value exceeding 0.12.

According to a second aspect of the invention a method for producing an enamelling steel sheet according to the first aspect of the invention is provided, wherein the steel sheet after hot rolling and cold rolling, wherein the steel sheet is rolled to a thickness between 0.10 mm and 0.34 mm, is continuous annealed at a temperature of at most 780° C. By continuous annealing to hot and cold rolled steel sheet at a temperature of at most 780° C the hydrogen retention of the steel is improved. Due to this improved hydrogen retention, fish scaling defects are avoided.

Preferably, the continuous annealing is performed at a temperature between 620 and 720° C. Below 550° C the steel is too hard for efficient (coil to coil) processing.

According to a third aspect of the invention the use of the enamelling steel sheet according to the first aspect of the invention is provided for the production of whiteboards and/or solar cell substrates and/or flat enamelled building panels. It has been found that the thinner gauges that can be produced according to the invention are very suitable for whiteboards, solar cell substrates and flat enamelled building panels. For these purposed, the steel sheet has not to be deformed or deep drawn.

The invention will be explained according to some embodiments of the invention.

Cold reduced enamelling steel sheet can be produced by preparing a suitable steel melt and casting the melt into a slab. The production process can include operations of hot rolling the slab, pickling the rolled product, cold rolling, annealing, and temper rolling.
For the trial use is made of three coils having the composition according to Table 1. The average tensile properties for thee coils are given in Table 2. Table 3 shows the picklability and fish scale sensitivity.

**Table 1 : all elements in ppm, Mn in mwt.%**

| | C | Mn | O | Al | Alₐₛ | B | N | B/N | Si | Cu | P | S |
|---|---|---|---|---|---|---|---|---|---|---|---|---|
| Coil 1 | 16 | 298 | 0 | 20 | 190 | 69 | 81 | 0.85 | 30 | 220 | 70 | 160 |
| Coil 2 | 16 | 298 | 0 | 20 | 190 | 69 | 81 | 0.85 | 30 | 220 | 70 | 160 |
| Coil 3 | 35 | 302 | 0 | 22 | 220 | 67 | 86 | 0.78 | 30 | 240 | 80 | 160 |

**Table 3: Picklability and fish scale sensitivity**

| | Picklability | Fishscale sensitive* |
|---|---|---|
| Coil 1 | OK | N |
| Coil 2 | OK | N |
| Coil 3 | OK | N |

| | | |
|---|---|---|
| * test criteria according to norm EN 10209. | | |

The coils have been produced in a continuous caster, then hot rolled, pickled, cold rolled and continuous annealed. Continuous annealing has been performed at a maximal average temperature of 680° C. Thereafter, temper rolling has been performed with a reduction of 1.2%.

The thickness of the enamelling steel strip thus produced is 0.285-0.305 mm The hardness measured is 90-110 in (micro)Vickers hardness. No fish scaling defects are observed during vitreous enamel application tests using special fish scale sensitive vitreous enamel according to the procedure described in norm EN 10206.

In coil 1 and coil 2 the grain size is found to be 9.5 units according to ASTM. For coil 3 the grain size is found to be 10.5 units according to ASTM.

## Claims

1. Cold reduced enamelling steel sheet comprising (in weight ppm unless otherwise indicated) $5 \leq C \leq 90 ;$ $0.10 \leq Mn \leq 0.50 \left(wt . %\right) ;$ ${Al}_{as} \leq 300 \left(acid soluble Al\right) ;$ $O \leq 35 ;$ $S \leq 350 ;$ $30 \leq N \leq 110 ;$ ${B}_{min} < B \leq {B}_{max} ;$ wherein ${B}_{min} = N \times 0.80 \times 10.8 / 14 {and B}_{max} = N \times 10.8 / 14 + 144 / 6 ;$ $50 \leq P \leq 160 ;$ in combination with ${Cu}_{min} \leq Cu \leq {Cu}_{max} ;$ wherein ${Cu}_{min} = P \times 1.00 \times 63.6 / 31 {and Cu}_{max} = P \times 2.00 \times 63.6 / 31 ;$ and optionally $Si \leq 190 ;$ the balance being Fe and inevitable impurities,
wherein the steel sheet has been continuous annealed, and
wherein the steel sheet has a thickness between 0.10 mm and 0.34 mm.

2. Steel sheet according to claim 1, wherein the steel sheet has a thickness between 0.12 and 0.34 mm, preferably between 0.15 mm and 0.32 mm, more preferably between 0.20 mm and 0.30 mm.

3. Steel sheet according to claim 1 or 2, wherein the steel has a maximal hardness of 85 - 130 micro Vickers with a load of 500 gram.

4. Steel sheet according to any one of the preceding claims, wherein Bₘₐₓ = N×10.8/14 + 83/6.

5. Steel sheet according to any one of the preceding claims, wherein Bₘᵢₙ = N×0.90×10.8/14, and preferably Bₘᵢₙ = N×1.00×10.8/14.

6. Steel sheet according to any one of the preceding claims, wherein 45 ≤ N ≤ 110 or wherein 30 ≤ N < 89.

7. Steel sheet according to claim 6, wherein Bₘₐₓ = N×1.20×10.8/14.

8. Steel sheet according to any one of the preceding claims, wherein Cuₘₐₓ = P×1.50×63.6/31.

9. Steel sheet according to any one of the preceding claims, wherein the maximum amount of C is 30 ppm by weight.

10. Steel sheet according to any one of the preceding claims, wherein the grain size according to ASTM is 11 units or less.

11. Steel sheet according to any one of the preceding claims, wherein the yield strength is between 140 MPa and 300 MPa, the tensile strength is between 270 MPa and 450 MPa, and the elongation to fracture is at least 30 %.

12. Method for producing an enamelling steel sheet according to any one of the preceding claims, wherein the steel sheet after hot rolling and cold rolling, wherein the steel sheet is rolled to a thickness between 0.10 mm and 0.34 mm, is continuous annealed at a temperature of at most 780° C.

13. Method according to claim 12, wherein the continuous annealing is performed at a temperature between 620 and 720° C.

14. Use of the enamelling steel sheet according to any one of the claims 1 - 11 for the production of whiteboards and/or solar cell substrates and/or flat enamelled building panels.

## Patentansprüche

1. Kältereduziertes emaillierendes Stahlblech, umfassend (in Gewichts-ppm, sofern nicht anders angegeben) $5 \leq C \leq 90 ;$ $0,10 \leq Mn \leq 0,50 \left(Gew . - %\right) ;$ ${Al}_{as} \leq 300 \left(säurelösliches Al\right) ;$ $O \leq 35 ;$ $S \leq 350 ;$ $30 \leq N \leq 110 ;$ ${B}_{min} < B \leq {B}_{max} ;$ wobei ${B}_{min} = N \times 0,80 \times 10,8 / 14 {und B}_{max} = N \times 10,8 / 14 + 144 / 6 ;$ $50 \leq P \leq 160 ;$ in Kombination mit ${Cu}_{min} \leq Cu \leq {Cu}_{max} ;$ wobei ${Cu}_{min} = Px 1,00 x 63,6 / 31 {und Cu}_{max} = P \times 2,00 \times 63,6 / 31 ;$ und optional $Si \leq 190 ;$ wobei der Rest Fe und unvermeidbare Unreinheiten sind,
wobei das Stahlblech durchgehend geglüht worden ist, und
wobei das Stahlblech eine Dicke zwischen 0,10 mm und 0,34 mm aufweist.

2. Stahlblech nach Anspruch 1, wobei das Stahlblech eine Dicke zwischen 0,12 und 0,34 mm, bevorzugt zwischen 0,15 mm und 0,32 mm, bevorzugter zwischen 0,20 mm und 0,30 mm aufweist.

3. Stahlblech nach Anspruch 1 oder 2, wobei der Stahl eine maximale Härte von 85-130 Mikro-Vickers mit einer Last von 500 Gramm aufweist.

4. Stahlblech nach einem der vorhergehenden Ansprüche, wobei Bₘₐₓ = Nx10,8/14 + 83/6.

5. Stahlblech nach einem der vorhergehenden Ansprüche, wobei Bₘᵢₙ = N×0,90× 10,8/14, und bevorzugt Bₘᵢₙ = N×1,00×10,8/14.

6. Stahlblech nach einem der vorhergehenden Ansprüche, wobei 45 ≤ N ≤ 110 oder wobei 30 ≤ N ≤ 89.

7. Stahlblech nach Anspruch 6, wobei Bₘₐₓ = N×1,20×10,8/14.

8. Stahlblech nach einem der vorhergehenden Ansprüche, wobei Cuₘₐₓ = P×1,50×63,6/31.

9. Stahlblech nach einem der vorhergehenden Ansprüche, wobei die maximale Menge an C 30 ppm nach Gewicht beträgt.

10. Stahlblech nach einem der vorhergehenden Ansprüche, wobei die Korngröße gemäß ASTM 11 Einheiten oder weniger ist.

11. Stahlblech nach einem der vorhergehenden Ansprüche, wobei die Streckgrenze zwischen 140 MPa und 300 MPa beträgt, die Zugfestigkeit zwischen 270 MPa und 450 MPa beträgt und die Bruchdehnung mindestens 30 % beträgt.

12. Verfahren zur Herstellung eines emaillierenden Stahlblechs nach einem der vorhergehenden Ansprüche, wobei das Stahlblech nach dem Warmwalzen und Kaltwalzen, wobei das Stahlblech zu einer Dicke zwischen 0,10 mm und 0,34 mm gewalzt wird, bei einer Temperatur von höchstens 780 °C durchgehend geglüht ist.

13. Verfahren nach Anspruch 12, wobei das durchgehende Glühen bei einer Temperatur zwischen 620 und 720 °C durchgeführt wird.

14. Verwendung des emaillierenden Stahlblechs nach einem der Ansprüche 1-11 für die Herstellung von Weißwandtafeln und/oder Solarzellsubstraten und/oder flachen emaillierten Bauplatten.

## Revendications

1. Tôles d'acier pour émaillage réduite à froid (en ppm de poids sauf indication contraire) $5 \leq C \leq 90 ;$ $0,10 \leq Mn \leq 0,50 \left(% en poids\right) ;$ ${Al}_{as} \leq 300 \left(Al soluble en milieu acide\right) ;$ $O \leq 35 ;$ $S \leq 350 ;$ $30 \leq N \leq 110 ;$ ${B}_{min} < B \leq {B}_{max} ;$ où ${B}_{min} = N \times 0,80 \times 10,8 / 14 {et B}_{max} = N \times 10,8 / 14 + 144 / 6 ;$ $50 \leq P \leq 160 ;$ en association avec ${Cu}_{min} \leq Cu \leq {Cu}_{max} ;$ où ${Cu}_{min} = P \times 1,00 \times 63,6 / 31 {et Cu}_{max} = P \times 2,00 \times 63,6 / 31 ;$ et éventuellement $Si < 190 ;$ le reste étant constitué de Fe et d'impuretés inévitables,
ladite tôle d'acier ayant été recuite en continu, et
ladite tôle d'acier possédant une épaisseur comprise entre 0,10 mm et 0,34 mm.

2. Tôle d'acier selon la revendication 1, ladite tôle d'acier possédant une épaisseur comprise entre 0,12 et 0,34 mm, de préférence entre 0,15 et 0,32 mm, idéalement entre 0,20 et 0,30 mm.

3. Tôle d'acier selon la revendication 1 ou 2, ledit acier possédant une dureté maximale de 85 à 130 microvickers avec une charge de 500 grammes.

4. Tôle d'acier selon l'une quelconque des revendications précédentes, où Bₘₐₓ = N×10,8/14 + 83/6.

5. Tôle d'acier selon l'une quelconque des revendications précédentes, où Bₘᵢₙ = N×0,90×10,8/14 et de préférence Bₘᵢₙ = N×1,00×10,8/14.

6. Tôle d'acier selon l'une quelconque des revendications précédentes, où 45 ≤ N ≤ 110 ou 30 ≤ N ≤ 89.

7. Tôle d'acier selon la revendication 6, où Bₘₐₓ = N×1,20×10,8/14.

8. Tôle d'acier selon l'une quelconque des revendications précédentes, où Cuₘₐₓ = P×1,50×63,6/31.

9. Tôle d'acier selon l'une quelconque des revendications précédentes, ladite quantité maximum de C étant de 30 ppm en poids.

10. Tôle d'acier selon l'une quelconque des revendications précédentes, ladite taille de grain selon la norme ASTM étant inférieure ou égale à 11 unités.

11. Tôle d'acier selon l'une quelconque des revendications précédentes, ladite limite d'élasticité étant comprise entre 140 MPa et 300 MPa, ladite résistance à la traction étant comprise entre 270 MPa et 450 MPa, et ledit allongement à la rupture étant supérieur ou égal à 30 %.

12. Procédé destiné à la production d'une tôle d'acier pour émaillage selon l'une quelconque des revendications précédentes, ladite tôle d'acier après laminage à chaud et laminage à froid, ladite tôle d'acier étant laminée jusqu'à une épaisseur comprise entre 0,10 et 0,34 mm, étant recuite en continu à une température inférieure ou égale à 780°C.

13. Procédé selon la revendication 12, ledit recuit en continu étant effectué à une température comprise entre 620 et 720°C.

14. Utilisation de la tôle d'acier pour émaillage selon l'une quelconque des revendications 1 à 11 pour la production des tableaux blancs et/ou des substrats de cellule solaire et/ou des panneaux de construction émaillés plats.
